

## UNITED STATES PATENT OFFICE

2,084,532

PROCESS OF PREPARING STEAM  
CYLINDER OIL

Arthur Lazar, Associated, and Joseph V. Crenna,  
Concord, Calif., assignors to Associated Oil  
Company, San Francisco, Calif., a corporation  
of California

No Drawing. Application May 29, 1936, Serial  
No. 82,548

8 Claims. (Cl. 87—9)

This invention relates to the treatment of lubricating oil to insure stability under conditions of high temperatures and pressures in the presence of steam and has for a particular object the preparation of a lubricating oil especially adapted to function in the cylinders of steam engines.

In the manufacture of steam cylinder oils certain specifications must be strictly adhered to because of operating conditions peculiar to the uses of such oils.

Steam cylinder oils may not be supplied to the walls of the pistons and cylinders of the engine in many of the well-known forms of lubrication, but are introduced to the cylinder with the steam in such fashion that they are finely divided by atomization, whereby they are spread evenly over the moving parts.

In modern steam engine practice the temperature of the steam in the cylinder of the engine when closed by the piston goes as high as 500° F. under its corresponding pressure, and under such conditions it is highly important not only that a proper distribution of the oil is assured, but also that the stability of the oil is such as to resist decomposition, whereby undesirable deposits, such as coke, and the like, are eliminated.

Oils which have a tendency to emulsify with steam are best suited for steam cylinder oils and heretofore it has been common practice to compound with a mineral oil a certain percentage of a fatty oil, such as tallow, which causes emulsification. Such fatty oil, or oils, usually represent up to 8% to 10% of the mineral oil, but in addition to being costly, are decomposed at high temperatures which do not affect the mineral oil hydrocarbons, thus forming free fatty acids which attack metals under such temperature conditions.

The problems of steam cylinder lubrication are thus inherently different from the problems of lubricating the cylinders of internal combustion engines, due to operating conditions at high temperatures and pressures in the presence of water vapor, which factors require that the cylinders be preferentially wet with the oil rather than with the water.

For this reason, high viscosity oils have been found best suited for steam cylinder lubrication and such oils should be processed for emulsification with the steam used in order to provide the desired preferential wetting of the cylinder with oil.

Generally speaking, the range of high viscosities for such a steam cylinder oil may be between 1000 and 10000 secs. S. U. at 100° F. and preferably between 1500 and 6000 secs. These figures

may vary depending on whether a Pennsylvania oil or a western oil is used but the viscosity of a steam cylinder oil is generally greatly different from a transformer oil, or light lubricating oil used in internal combustion engines.

This invention provides a way of insuring the stability of steam cylinder oils while emulsifying the same under operating conditions, which is preferably accomplished in the following manner.

As a base stock for steam cylinder oils it is preferred to select a lubricating oil of high viscosity which is composed mainly of saturated hydrocarbons, such oil, for example, being a heavy asphaltic base, or mixed base, oil, which is highly refined by treatment with liquid sulphur dioxide, as in the well-known Edeleanu process, to remove unsaturated hydrocarbons, aromatics, etc. Such lubricating oil, thus treated, shows the greatest stability under high heat conditions, but, of course, a body of saturated hydrocarbons may also be prepared by extensive sulphuric acid treatment, or even distilled from certain stocks, such as Pennsylvania crudes.

To such stable lubricating oil is added a trace of a lime or magnesium soap of an organic acid, such, for example, as oleic acid, stearic acid, naphthenic acid, or sulphonic acid, the proportion of such added soap ranging in very small percentages of the oil, preferably from .01% to 1%.

While the above-mentioned soaps are preferred, the use of minute quantities of other soaps is effective to give emulsifying properties to lubricating oils, the percentages being such that the amount of ash arising from their use as emulsifiers is generally too small to be determined analytically.

This use results in a steam cylinder oil of unimpaired stability which emulsifies sufficiently to get the desired distribution, the soaps being easily combined with the saturated hydrocarbons due to their oil solubility.

Likewise, a steam cylinder oil having the required emulsifying properties may be prepared from oils which result from the distillation of a suitable crude stock and which may be naturally composed mainly of saturated hydrocarbons. For instance, residual oils of Pennsylvania origin are found to contain organic acids in sufficient quantities that when traces of oxides, or hydroxides, are added to the oil when heated, such oil develops the desired pronounced emulsifying properties.

A preferred amount of magnesium oxide, or lime, or other alkaline earth oxide, or hydroxide,

which may be added to such residual oil varies from .01% to 1%, and such is incorporated in the oil by intimate mixing at elevated temperatures, preferably about 300° F., and generally in excess of atmospheric temperatures. This oil may then be used as straight steam cylinder oil, or may be blended in amounts of from 10% to 20% with a body of a highly refined oil of high stability, such as the SO<sub>2</sub> treated oil previously described.

While it is unnecessary, the use of small amounts of an acidless fatty oil with the steam cylinder oils prepared as above described, has sometimes a beneficial effect in lowering the surface tension, but the quantity used, from 0% to 3%, is kept as low as possible and in any event is far less than the amount normally used in compounding steam cylinder oils.

This application is a continuation in part of our co-pending application S. N. 492,615, filed Oct. 31, 1930.

We claim:

1. A process of preparing an emulsifiable oil suitable for use in the cylinders of steam engines which comprises: adding from 0.01% to 0.1% of an alkaline earth metal soap of an organic acid normally present in petroleum to a hydrocarbon lubricating oil having a viscosity suitable for use as a steam cylinder oil; said oil being substantially free from organic acids.

2. A process of preparing an emulsifiable oil suitable for use in the cylinders of steam engines which comprises: adding from 0.01% to 0.1% of an alkaline earth metal soap of an organic acid normally present in petroleum to a saturated hydrocarbon lubricating oil having a viscosity suitable for use as a steam cylinder oil; said oil being substantially free from organic acids.

3. A process of preparing an emulsifiable oil suitable for use in the cylinders of steam engines which comprises: adding from 0.01% to 0.1% of an oil soluble alkaline earth metal soap of an organic acid normally present in petroleum to a hydrocarbon lubricating oil having a viscosity suitable for use as a steam cylinder oil; said oil being substantially free from organic acids.

4. A process of preparing an emulsifiable oil suitable for use in the cylinders of steam engines, which comprises: mixing a percentage of an alkaline earth metal soap of an organic acid normally present in petroleum to a hydrocarbon

lubricating oil having a viscosity suitable for use as a steam cylinder oil and being substantially free from organic acids; said percentage ranging upward from 0.01% to a percentage insufficient to deposit ash when said mixture is injected with direct steam into the cylinder of a steam engine.

5. A process of preparing an emulsifiable oil suitable for use in the cylinders of steam engines which comprises: mixing a percentage of calcium naphthenate to a hydrocarbon lubricating oil having a viscosity suitable for use as a steam cylinder oil and being substantially free from organic acids; said percentage ranging upward from 0.01% to a percentage insufficient to deposit ash when said mixture is injected with direct steam into the cylinders of a steam engine.

6. A process of preparing an emulsifiable oil suitable for use in the cylinders of steam engines which comprises: mixing a percentage of magnesium naphthenate to a hydrocarbon lubricating oil having a viscosity suitable for use as a steam cylinder oil and being substantially free from organic acids; said percentage ranging upward from 0.01% to a percentage insufficient to deposit ash when said mixture is injected with direct steam into the cylinders of a steam engine.

7. In the lubrication of the cylinders of steam engines, the improvement which comprises commingling with the steam supplied to such cylinders: a hydrocarbon lubricating oil substantially free of organic acids and containing upward of 0.01% of an alkaline earth metal soap of organic acids normally present in petroleum sufficient to cause emulsification of said oil when introduced into said cylinders but insufficient to cause substantial formation of decomposition products at the temperature of such emulsification.

8. In the lubrication of the cylinders of steam engines, the improvement which comprises commingling with the steam supplied to such cylinders: a hydrocarbon lubricating oil substantially free of organic acids and containing from 0.01% to 0.1% of an alkaline earth metal soap of organic acids normally present in petroleum sufficient to cause emulsification of said oil when introduced into said cylinders but insufficient to cause substantial formation of decomposition products at the temperature of such emulsification.

ARTHUR LAZAR.

JOSEPH V. CRENNAN.

50